

## UNITED STATES PATENT OFFICE

HARRY F. PORTER, OF TRENTON, NEW JERSEY

## METHOD OF PRODUCING AND REFINING ALLOYS

No Drawing. Original application filed January 20, 1927, Serial No. 162,245. Divided and this application filed September 28, 1928. Serial No. 309,087.

My invention relates to a ternary alloy, and more particularly to a method of producing and refining a ternary alloy.

My invention resides in a method of producing and refining a ternary alloy of copper-nickel and iron.

My invention further resides in a method of refining a copper-nickel-iron alloy for use as a magnetic alloy wherein copper having an appreciable oxygen content is utilized to effect reduction of carbon in the alloy.

My invention further resides in a method of the character hereinafter described and claimed.

15 In my researches, I have found that a magnetic alloy may be made of copper, nickel and iron within the limits of

Per cent  
20 Copper ..... 3-10  
Nickel ..... 35-55  
Iron ..... 35-55  
which in certain fields of application is electrically and magnetically superior to known magnetizable substances and processes the 25 additional mechanical advantage of being easily worked, as is hereinafter more fully described.

The alloy per se and electro-magnetic devices utilizing it are claimed in my co-pending application Serial No. 162,245 filed January 20, 1927, of which this application is a division.

The preferred method of making this ternary alloy consists of placing a quantity of 35 manganese or manganese and magnesium in the bottom of the silica or quartz crucible of an induction furnace and superimposing upon it the proper proportion of copper. In lieu of this arrangement, an alloy of copper and manganese, or of copper and magnesium, or of copper, manganese and magnesium, is employed. In any case, the iron and nickel, preferably in the form of sheets alternately arranged, are placed above the copper 40 mixture or alloy so that the latter, which melts first, in effect forms a solvent in which the iron and nickel dissolve. The downward movement of these melting metals and the currents induced by the primary winding of 45 the furnace cause a stirring action which re-

sults in a uniform mixture of the metals throughout the entire mass.

To obtain the desired magnetic properties of the alloy, the total carbon content should not exceed .1 of 1% by weight of the alloy 55 and should be preferably below .05%. In making the alloy the nickel should contain but little carbon, less than .005%. Electrolytic nickel may be used. Manganese one-half of 1% insures removal of sulphur from 60 the nickel and also deoxidizes it. The iron should be of high purity, containing from but .01% to .03% carbon. The copper, which may be of the usual commercial varieties, is of high oxygen content and refines 65 from the iron the small traces of carbon that may be present. By arranging the materials in the furnace as described, the melting and refining operations proceed simultaneously. The alloy should be poured soon after the 70 entire mass has become molten; otherwise gases are formed which produce porous bars or castings.

An important advantage of my refining operation is that metals obtainable commercially, may be utilized in such operation, thereby greatly reducing the cost thereof. Commercial copper generally contains an appreciable amount of oxygen in the form of copper oxide, while commercial ingot iron 80 necessarily contains a small amount of carbon; an amount too high, however, for use in highly sensitive magnetic alloys. When the copper in the bottom of the crucible has melted, and as the iron which is of greater 85 weight, gradually dissolves and settles in the copper solvent, the oxygen present in the copper effects reduction of the carbon in the iron. Cold copper has higher specific gravity than cold iron, but when molten the action is as described above. By such method, it is possible to utilize commercial ingot iron instead of electrolytic iron, which although more expensive, has been previously used to a great extent for highly sensitive magnetic 95 alloys. For the combination of 46½% nickel, 46½% iron and the balance of copper, except for small amounts of manganese, magnesium and traces of the usual impurities, the melting point of the alloy is about 100

1300° centigrade and the time of melting a charge depends, of course, upon the amount of material, and other variables.

The alloy may be cast in various shapes, by the use of cast iron or sand moulds and thereafter machined. After all of the mechanical operations have been performed, the castings are annealed in a reducing or neutral atmosphere, free from all traces of carbon, sulphur or oxygen, at temperatures ranging from 900° to 1200° centigrade, the time of holding and temperature being dependent on the thickness of the piece and also the desired magnetic characteristics. The metal before annealing is, to all practical purposes, non-magnetic.

The castings may be annealed in air if the precaution is taken to cover them with some substance such as iron borings, to remove impurities from the furnace gases before they come in contact with the casting. Further, during the cooling down in the open air, a partial vacuum is produced, sucking in air, which, except for the presence of the filter, as of iron borings, would oxidize the castings. As a matter of fact, the results produced by surrounding the casting with iron filings and annealing in air are fully as satisfactory as those produced by annealing in an atmosphere of hydrogen, which is considerably more expensive than the iron filing anneal. The hydrogen anneal is very commonly used for highly sensitive magnetic metals, or alloys having no copper in their composition. In general, the higher the temperature at which the annealing is performed within the range given, the less the time required to attain the desired objective.

The magnetic characteristics of the alloy are such that when a casting of the metal is used as a core or other magnetic element in electro-magnetic devices and the like, as transformers, alternating current relays, its performance compares favorably with a laminated core of the usual known magnetic alloys, as silicon-steel.

Instead of casting the metal in molds substantially of the shape and size of the finished product it may be poured in flat slabs similar to the practice employed with non-ferrous metals prior to rolling. The bars or slabs are very malleable, and may be either hot or cold rolled, preferably cold rolled so as to reduce to a minimum the absorption of carbon, oxygen or sulphur during the rolling, inasmuch as any of these impurities are detrimental to the final desired magnetic qualities of the alloy. It is almost impossible to safeguard against this "poisoning" of the metal during the much more involved and expensive hot rolling process which is employed with the known magnetic substances. The cold rolling also effects a change in the internal structure of the alloy

such that an examination under the microscope of a cross-section of the cold rolled metal reveals a series of minute, finely separated laminae.

This undoubtedly is explanatory of the low, eddy current losses of the alloy when cold rolled in the form of strips since each lamination or strip is in itself a plurality of thinner laminations. A similar condition results to a lesser degree if a casting of the material is subjected to a slight rolling consisting of a few passes.

After all mechanical operations have been completed, the strips are annealed as previously described. The tendency of light strips to stick together during the annealing process, if stacked and subjected to temperatures in excess of 925° C. may be minimized by giving the strips a light surface oxidation prior to annealing. When annealed in a reducing atmosphere the material assumes a high lustre and when air annealed takes on an oxide coating desirable for transformer or other construction in which a core is built of a pile of laminations.

The alloy may also be poured in round ingots, which are readily drawn into a wire which in turn may be drawn down to the finest sizes. After annealing, the wire may be insulated and employed in circuits, as radio frequency circuits, wherein high permeability and low losses at feeble inductions are desirable. If cold drawn, the rod or wire is striated, and is, in effect, a bundle of very fine, substantially parallel wires or rods.

The magnetic properties of the alloy render it particularly useful in electro-magnetic devices involved in the transmission of currents of sound frequency, such as for example audio-transformers and impedances, having a magnetic member or members subjected to an alternating flux whose frequency may vary from 10 to 10,000 cycles per second, superimposed upon a relatively large biasing magneto-motive force.

What I claim is:

1. The method of producing a magnetic alloy which comprises melting a predetermined amount of copper containing copper oxide to form a solvent, melting and dissolving predetermined amounts of nickel and iron in said solvent, and effecting reduction of carbon in said alloy by the copper oxide.

2. The method of producing a magnetic alloy which comprises melting a predetermined amount of commercial copper containing copper oxide to form a solvent, melting and dissolving predetermined amounts of nickel and commercial ingot iron in said solvent, and effecting reduction of carbon in said iron by the copper oxide.

3. The method of simultaneously produc-

ing and refining a copper-nickel-iron alloy which comprises melting by induced electric currents a predetermined amount of copper having relatively high oxygen content, melting and dissolving a predetermined amount of nickel and commercial iron in said melt, effecting reduction of carbon in said iron by the oxygen content of the copper, and effecting a stirring motion of said solution to insure uniformity thereof by said induced currents.

4. The method of producing and refining a copper-nickel-iron alloy which comprises placing copper containing appreciable oxygen content in the bottom of a crucible, superimposing nickel, and iron containing low carbon content, on said copper, melting said copper to form a solvent, melting and dissolving the nickel and iron in said solvent, and effecting reduction of the carbon content of the iron as the heavier metals melt and commingle with said solvent.

HARRY F. PORTER.

25

30

35